

July 13, 1937.

J. FLETCHER

2,086,862

WALLBOARD

Filed Aug. 22, 1935



Fig. 1



Fig. 2

INVENTOR  
John Fletcher  
by Parker, Rocknow & Turner  
ATTORNEYS

## UNITED STATES PATENT OFFICE

2,086,862

## WALLBOARD

John Fletcher, Kenmore, N. Y., assignor to Plas-  
tergon Wall Board Company, Buffalo, N. Y., a  
corporation of New York

Application August 22, 1935, Serial No. 37,351

12 Claims. (Cl. 91—68)

This invention relates to wallboard, and particularly to a composition wallboard having as a part thereof a sheet of open pore fiber insulating board. Heretofore, attempts have been made to apply a plastic gypsum mixture to a face of such open pore fiber insulating board, but the product obtained has been unsatisfactory because it has been impossible to avoid cracking of the gypsum coating during handling of the sheet, and because of the unequal expansion and contraction of the coating and open pore board. The gypsum mixtures heretofore used for this purpose have been brittle, with a tendency to disintegrate and separate from the porous and fibrous surface of the open pore board during transportation and handling, prior to and during the application of the board to a wall construction. A gypsum surface or face on a wallboard is often very desirable, but because of the expansion and contraction of the fiberboard, it is also difficult to keep the cracks between abutting edges of adjacent sheets of such board filled with a gypsum mixture so as to form a continuous union between the gypsum coatings on the adjacent or abutting sheets. When the sheets contract, the filling tends to separate from the edge of one sheet or the other and form an objectionable crack in the gypsum surface or coating.

An object of the invention is to provide an improved wallboard which will have a gypsum finished surface, with which the development of cracks and disintegration during handling of the board will be substantially prevented, with which separation of the gypsum coating or finish from the board will be substantially prevented, which will have maximum strength, rigidity and durability, which will have substantial resistance to destructive insects, and which will be relatively simple, and inexpensive.

Another object of the invention is to provide an improved wallboard having a gypsum coating or finish, with which the cracks between abutting edges of adjacent sheets as applied to a wall construction, may be filled with a gypsum mixture to provide a continuous gypsum surface from one sheet to the other, with which the development of cracks in the gypsum coating or finish at the abutting edges of the sheets will be substantially reduced or prevented, and with which greater adhesion between the crack filler and the boards may be obtained.

Another object of the invention is to provide an improved method of making wallboard, which will produce a superior wallboard having a gypsum coating or finish, maximum strength, mini-

mum expansion and contraction when assembled as part of a wall construction, and with which the cracks between abutting edges of adjacent sheets may be easily filled in a manner to seal the cracks and provide a durable, continuous gypsum finish from one sheet to the other.

Various other objects and advantages will be apparent from the following description of examples of the invention, and the novel features will be particularly pointed out hereinafter in connection with the appended claims.

In the accompanying drawing:

Fig. 1 is a sectional elevation through a portion of a sheet of wallboard constructed in accordance with this invention; and

Fig. 2 is a sectional elevation through a part of a wall construction utilizing this improved board, and illustrating the manner of filling the cracks and forming a continuous gypsum finish between adjacent sheets of said board.

In accordance with this invention I impregnate a sheet of open pore fiber insulating board with a suitable stiffening agent, and then apply to a face of such board a plastic coating containing calcined gypsum and an adhesive, so that the adhesive of the coating will adhere firmly to the stiffened board. By impregnating the board with a stiffening agent, its expansion and contraction is greatly restricted, which reduces the tendency of the gypsum coating to crack or separate from the board. Preferably, I impregnate a sheet of open pore fiber insulating board with a readily soluble stiffening resin, and this impregnation, in some instances, is preferably distributed throughout substantially the entire board, although some of the desirable results may be obtained to some extent through impregnation only of a surface layer of the board.

I prefer to carry out the impregnation by applying to the board a solution of the resin in a volatile solvent, because I have found that by using the resin solution, great strength and rigidity of the board is obtained. To a face of this board, which should be an impregnated face, I apply the coating of a plastic mass containing calcined gypsum with an adhesive, and the most satisfactory adhesives are resinous solutions containing a solvent for the resin with which the fiberboard is impregnated. The inclusion in the gypsum mixture of a quantity of fibrous, non-metallic minerals such as fibrous types of amphibole, serpentine and chrysotile, is advantageous and adds materially to the strength and tenacity of the coating. When a plastic mass or mixture of calcined gypsum, with or without

added fibers, and such a resinous solution is applied to the impregnated board, the solvent in the resinous solution of the plastic mass, where it contacts with the impregnated board, will soften or partially dissolve the resinous impregnating agent of the board at approximately the surface of the board, and then when the solvent is evaporated or absorbed a very firm union between the coating and the board is obtained.

10 The resinous adhesive used in the gypsum mixture greatly increases the strength, durability, and rigidity of the gypsum coating, because it causes greater cohesion between the particles in the mixture of the coating. The board, because 15 of its impregnation with the resin, will be largely unaffected by atmospheric and temperature changes and, therefore, the tendency of the gypsum coating to crack or chip off during use will be reduced or prevented. The tendency of the 20 coating to crack and chip is also reduced by the fibrous non-metallic minerals which may advantageously be included with the gypsum in the coating mixture.

Among the resins which are suitable for impregnation of the fiberboard, as well as for mixture with the calcined gypsum forming the coating, may be particularly mentioned the natural resins such as shellac, rosin, gum accroids, manila gum and kauri gum, and among the synthetic resins may be particularly mentioned the phenol-aldehyde resins, the polybasic acid-polyhydric alcohol, fatty acid type of resins, and the urea-aldehyde type of resins. The solvent used for the resin with which the board is impregnated should preferably be a readily volatile solvent. Alcohol is a very satisfactory and inexpensive, yet volatile, solvent for this purpose.

As one example of the invention, a sheet of open pore fiber insulating board is thoroughly 40 impregnated with a solution of one of the above mentioned resins in alcohol. Then to a face of such an impregnated sheet I apply a coating, in plastic form, which may be prepared as follows:

45 Approximately 100 parts by weight of dry calcined gypsum is mixed with 50 parts of a resin solution containing 20 parts of shellac and 30 parts of alcohol. This plastic gypsum mass may be applied to a face of the impregnated board by trowel or brush and levelled out on the board. 50 The thickness of the coating may be whatever is desired, but I have found that it may vary for practical purposes between  $\frac{1}{64}$  of an inch to  $\frac{1}{8}$  of an inch without danger of the surface coating cracking. Preferably, the impregnated board is 55 dried somewhat after impregnation, although with a readily volatile solvent, sufficient air drying may occur after the impregnation before coating can be applied thereto.

60 The alcohol or other solvent in the gypsum plastic coat will, wherever it contacts with the fiber board, soften or partially dissolve the alcohol soluble resin with which the board was impregnated, and then as the plastic mass or coating hardens and the alcohol or solvent evaporates, 65 there will be a firm and unitary union between the resin of the gypsum coating and the resin with which the board is impregnated. In addition, the resin in the gypsum coating will increase the cohesion between the gypsum particles, and 70 thus provide a very hard gypsum finish or coating on the board which adheres to the board with a maximum of firmness. Any of the other resins may be employed in a similar manner, both for the impregnation of the board and for the preparation and application of the gypsum coating.

When the improved gypsum wallboard is applied to a wall construction, the sheets are usually secured to a wall or basic structure by nails driven through the board into the basic structure. In Fig. 2 I have illustrated a simple manner by 5 which this improved board may be attached to a basic structure without the objectionable feature of having the attaching nails visible on the exterior of the wall. Referring now to Fig. 2, the portion of a wall construction in which two sheets 10 of open pore, fiber insulating board that have been impregnated and coated with a gypsum finish or coating in accordance with this invention, are brought together against a basic structure 12 so as to approximately abut edge to edge and 15 lie flat against the basic structure 12 along the abutting edges of the improved board.

A plurality of nails 13 may then be driven through the sheets 10 into the basic structure 12 at the abutting edges of the sheets, the nails 20 being preferably started adjacent the base of the coatings and driven somewhat diagonally through the impregnated open pore fiberboard sheets 10 into the basic structure 12, as shown clearly in Fig. 2. With this arrangement the 25 nails will not pass through the gypsum finish or coatings on the improved board, but largely through the impregnated basic sheets 10. Since the impregnated sheets now have greater 30 strength and rigidity, it is possible to pass the nails through the end edges of the impregnated sheets and still obtain a satisfactory attachment between the board and the basic structure 12.

The crack or space between the adjacent edges of the improved wallboard may then be filled 35 with a plastic mass 14, which preferably should contain calcined gypsum mixed with an adhesive such as a resinous solution containing a solvent for the resin with which the sheets 10 are impregnated, and therefore the mass 14 may advantageously be of the same plastic composition as that of the gypsum coating 11 on the impregnated board. The solvent in the plastic mass will soften, and form a firm union with, the resin with which the open pore sheets 10 are impregnated and also the resin of the coatings 11. If 40 it becomes necessary to drive attaching nails 15 through a face of the coated sheets, the nails are preferably countersunk at their heads and the countersunk holes 16 then filled with a plastic mass similar to the crack filler 14.

It will be understood that various changes in the details and materials, which have been herein described and illustrated in order to explain the nature of the invention, may be made by those 55 skilled in the art within the principle and scope of the invention as expressed in the appended claims.

I claim as my invention:

1. An improved wallboard comprising a sheet 60 of open pore, fiber insulating board impregnated with a stiffening resin solution, and having an adherent surface coating of a mixture containing calcined gypsum and a resin solution in which the impregnating resin is soluble.

2. An improved wallboard comprising a sheet 65 of open pore, fiber insulating board impregnated with an alcohol soluble stiffening agent, and having a hardened surface coating which has been applied thereto while plastic and containing calcined gypsum mixed with an alcohol-containing, resin solution, whereby the alcohol in the applied plastic coating will unite the coating firmly to the open pore board through the impregnating agent therein.

3. The method of making an improved wall-board which comprises impregnating a sheet of open pore, fiber insulating board with a solution of a stiffening resin in a volatile solvent, then applying to a face of said impregnated sheet a plastic coating containing calcined gypsum mixed with a resinous solution in which the impregnating resin is soluble, whereby when the plastic coating hardens the resin intermixed therewith increases the cohesion between the gypsum particles and the solution in the plastic coating will soften and form a firm union with the resin impregnating the fiberboard.

4. The method of making an improved wall-board which comprises impregnating a sheet of open pore, fiber insulating board with a solution of a stiffening resin in a volatile solvent, substantially drying the impregnated board to harden the resin therein, and then applying to a face of the impregnated sheet a plastic coating containing a mixture of calcined gypsum with a resinous solution in which the impregnating agent is soluble, and then hardening the coating, whereby the resin intermixed with the gypsum will increase the cohesion between the gypsum particles and the solution intermixed with the resin will soften and form a union between the resin-containing coating and the impregnating resin of the sheet.

5. The method of preparing an improved wall-board which comprises impregnating a sheet of open pore, fiber insulating board with an alcohol solution of a stiffening resin, and then applying to a face of the impregnated sheet a coating of a plastic mass containing a mixture of calcined gypsum with a resinous solution containing alcohol, and then hardening said coating.

6. The method of preparing an improved wall-board which comprises impregnating a sheet of open pore, fiber insulating board with a solution containing a stiffening resin, and then applying to a face of said impregnated sheet, a coating of a plastic substance containing a mixture of calcined gypsum with a resinous solution including alcohol, and then hardening said coating.

7. The method of preparing an improved wall-board which comprises impregnating a sheet of open pore, fiber insulating board with an alcohol-soluble stiffening resin, and then applying to a face of the impregnated sheet, a coating of a plastic mass containing calcined gypsum mixed

with a solution of shellac in alcohol, and then hardening said coating.

8. The method of making an improved wall-board which comprises impregnating a sheet of open pore, fiber wallboard with an alcohol soluble resin to stiffen said sheet, and then applying to a face of the impregnated sheet, a coating of a plastic mass containing calcined gypsum, shellac and alcohol approximately in the proportions of 100 parts by weight of dry calcined gypsum and 50 parts of a resin solution containing 20 parts of shellac and 30 parts of alcohol, and then hardening the coating.

9. An improved wallboard comprising a sheet of open pore, fiber insulating board impregnated with a stiffening resin which is soluble in a volatile solvent, and having on a face thereof, a coating containing a mixture of calcined gypsum with a resin solution containing a solvent for the impregnating resin, whereby said solvent in the coating mixture will soften and form a union with the impregnating resin in said sheet.

10. An improved wallboard comprising a sheet of open pore, fiber insulating board impregnated with an alcohol solution containing a stiffening resin, and having on a face thereof a coating of a mixture, applied while plastic, containing calcined gypsum intermixed with an alcohol solution of a resin, whereby the alcohol of the plastic coating will soften the impregnating resin of said sheet and form a firm union between the coating and the sheet.

11. An improved wallboard comprising a sheet of open pore, fiber insulating board having at least a surface layer thereof impregnated with a soluble resin, and having on said impregnated surface layer, an adherent coating, applied while plastic, containing a mixture of calcined gypsum with a resinous solution including a solvent for the impregnating resin of said sheet, whereby the solvent in said plastic coating will soften the impregnating resin on said surface layer of said sheet and form a firm union between it and the resin in said coating.

12. An improved wallboard comprising a sheet of open pore, fiber insulating board impregnated with a stiffening agent, and having on a surface thereof a coating, applied while plastic, containing a mixture of calcined gypsum and a solvent for said agent.

JOHN FLETCHER.